

Nov. 3, 1953

A. F. BURKARDT

2,657,717

PRESHRUNK YARN OR FABRIC

Filed Dec. 3, 1949

FIG. 2



FIG. 3



FIG. 4



FIG. 6



FIG. 5



FIG. 7



FIG. 1



FIG. 8



Inventor

Anton F. Burkardt

By

Van Patten & Shinsky  
Attorneys

## UNITED STATES PATENT OFFICE

2,657,717

## PRESHRUNK YARN OR FABRIC

Anton F. Burkhardt, New York, N. Y., assignor to  
Sativa Corporation, a corporation of New Jersey

Application December 3, 1949, Serial No. 130,933

1 Claim. (Cl. 139—426)

**1** This invention relates to a method of producing pre-shrunk yarns or fabrics and the products produced thereby and more particularly to such a method for producing pre-shrunk yarns or fabrics containing bast fibres. The term "pre-shrunk" applied to yarns and fabrics in this specification and claim means a yarn or fabric which is shrunken before fabrication to the extent herein described and which is therefore comparatively shrink-proof.

This process employs the use of pre-shrunk degummed bast fibres such, for example, as flax or hemp, which may be degummed as described in the copending application, Serial No. 103,262, filed July 6, 1949, in which is taught the art of degumming raw fibres and shrinking the same. A preferred form of raw fibre for treatment by the method described in the aforesaid copending application is described in the copending application, Serial No. 87,594, filed April 15, 1949.

No method or process has heretofore been known that would sufficiently degum and pre-shrink bast fibers to the extent necessary to produce the degummed and pre-shrunk fibrils disclosed herein in commercial quantity until the method of degumming and pre-shrinking disclosed in the co-pending application Serial No. 103,262 aforesaid was invented. This enabled flax and hemp to be dry-spun on ordinary cotton spinning machinery and eliminated wet spinning heretofore necessary.

As no sufficiently degummed and pre-shrunk bast fibrils were available, no pre-shrunk yarns or fabrics could be made, either solely of degummed and pre-shrunk fibrils or such fibrils blended with other shrinkable fibers, such as cotton or rayon. It is for this reason that no degummed pre-shrunk staples for dry spinning, such for example as linen, have ever been available to the textile trade. In this connection, it will be noted that degummed, pre-shrunk bast fibrils such as linen, for example, will not shrink more than 2%, and usually much less, when made into yarn and the yarn into fabric, while ordinary non-degummed hemp and flax (linen) as commonly used commercially, both alone and blended with other fibers, will shrink from 15% to 30%, depending upon the blend.

The century old method of linen fibre production which is today internationally practiced, produces only retted linen fibres, which are not degummed or shrunk. Such fibre, on account of the gum content, is too stiff to be spun on standard cotton or woolen machinery or for dry spinning. The yarns produced by retted linen fibre

are spun over special linen machinery by a wet spinning process to make the fibres soft and pliable, and the yarns or fabrics are later processed and degummed in yarn or fabric form. The resultant material however, is not shrink-proof.

The new method disclosed in the copending application, Serial No. 103,262 produces shrunk linen staples similar in staple length or fineness to cotton, which can be spun over standard cotton or woolen machinery. These fibre staples are as fine as 1½ denier, so that they can be blended with synthetic fibres or rayon or others, or with fine wool or natural fibres, by dry spinning over any conventional textile machinery, which has never been possible before or practiced in the textile industry.

Linen staples produced by known methods of retting and processing cannot be spun or blended with fine synthetics or natural fibres over standard textile machinery, nor will they reduce or eliminate the shrinkage of resulting yarns or fabrics, as is the case with shrunk linen produced under the process described in the aforesaid application, Ser. No. 103,262.

The instant invention is therefore directed to the use of fibrils of bast stalks that are degummed and pre-shrunk as taught in said application, Serial No. 103,262, or produced in any other suitable manner.

**30** The objects of the instant invention are:

(A) To produce a pre-shrunk roving composed wholly of bast fibres.  
(B) To produce a composite roving composed in part of pre-shrunk bast fibres and other fibres, either natural or synthetic.  
(C) To produce a yarn including (A) or (B) or a mixture of them.  
(D) To produce a fabric composed in whole or

**40** in part of (C).

The following specification and accompanying drawings illustrate the method herein disclosed and examples of preferred forms of staples and fabrics produced thereby. It will be understood, however, that what is herein disclosed is merely illustrative and not limitative, and that various modifications can be made, the invention being defined by the appended claim.

In the accompanying drawings:

**50** Figure 1 illustrates a sliver or roving composed wholly of bast fibres to produce the pre-shrunk roving as defined under object (A) hereof;

Figure 2 illustrates a composite sliver or roving composed in part of pre-shrunk bast fibres and

in part of other fibres to produce the roving as defined under object (B) hereof;

Figure 3 illustrates a composite yarn;

Figure 4 illustrates another composite yarn;

Figures 5 and 6 illustrate yarns as referred to under object (C) hereof; and

Figures 7 and 8 illustrate fabrics as referred to under object (D) hereof.

Referring to Fig. 1, if bast fibres are degummed to produce fibres of desired staple length and denier in a suitable degumming apparatus such as that for example described in the co-pending application, Serial No. 103,262 aforesaid, or in any other suitable manner, where natural fibres are degummed, boiled off and subjected to a rinse, the degummed washed fibre is pre-shrunk.

Under such treatment a web of natural fibre will shrink from a total length of 50 feet to 42 feet, and each fibril 10 thereof of course shrinks in proportion.

The pre-shrunk web may now be opened up and prepared for spinning. This produces individual fibrils 10 of pre-shrunk fibre and these may be from  $1\frac{1}{4}$  to  $2\frac{1}{2}$  inches long and may average  $1\frac{1}{2}$  denier. It will be observed that these fibres are obtained without cutting into predetermined lengths, and that the "opening up" process results in the production of "fibrils" as herein referred to.

As stated in the aforesaid application, Serial No. 103,262, the length of the fibrils can be predetermined by controlling the treatment of the raw fibre and, depending upon said treatment, may be made more or less receptive to standard dyes such as used for cotton, wool or synthetic fibres.

The fibrils 10 may now be formed into a sliver or roving 11 to be spun on standard existing textile machinery, and the resultant product will comprise a pre-shrunk roving composed wholly of bast fibres, which attains object (A) hereof and which may be used as hereinafter described.

Referring to Figure 2, the fibrils 10, instead of being made into a roving 11 composed wholly of them, are admixed with other fibres in any desired proportion to form a roving 12. This may be blended in any manner and may comprise:

1. A mixture of 50% by weight of bast fibres 10 and 50% cotton 13, or wool 14, or synthetic fibre 15, such as rayon.

2. Equal parts by weight of bast 10, wool 14, cotton 13 and rayon 15.

In all cases the fibrilla readily mix and form a composite roving which may be produced on standard existing textile machinery and which, by reason of the presence of the pre-shrunk bast fibrils 10 is substantially shrink-proof, the exact amount of shrinkage being determined by the admixture and the characteristics of the fibres 13, 14, 15 other than the pre-shrunk bast fiber 10 which prevents the yarns made from such roving from shrinking. This occurs because the degummed pre-shrunk fibers prevent the other shrinkable fibers from shrinking when interspun therewith, holding said shrinkable fibers against longitudinal shrinking.

Thus is produced a composite roving containing pre-shrunk bast fibers which attains object (B) hereof and which may be used as herein-after described.

Referring to Figure 3, a composite yarn is shown at 12a made of wool, pre-shrunk linen

75 (bast staples), rayon and cotton blended or mixed in any manner and proportions.

Referring to Figure 4, a composite yarn 16 is shown consisting of the pre-shrunk linen roving 11 (or the composite roving 12) and rovings of cotton 13a, wool 14a and rayon 15a.

Referring to Figure 5, a 2-ply yarn is shown consisting of a rayon roving 15a and the roving 11 (or 12).

Figure 6 shows a 2-ply yarn consisting of a wool roving 14a and the roving 11 (or 12).

Obviously the composition of the yarns, Figs. 5 and 6 can be varied within wide limits, but in all cases the presence of the pre-shrunk fibrils 10 in the yarn results in a pre-shrunk yarn which attains object (C) hereof.

A 4/1 yarn made as described herein and composed of rovings 11 has the following characteristics:

#### Comparative breaking strength

| Dry      | Wet      | Hot Wet  |
|----------|----------|----------|
| 316 lbs. | 510 lbs. | 726 lbs. |

130% increase normal to hot

Referring to Figure 7, the numeral 17 generally denotes a fabric including pre-shrunk yarn as previously described.

Now the extent of the use of such pre-shrunk yarn in the fabric may be varied within wide limits, and the pre-shrunk quality of the fabric may be varied accordingly.

Assuming for the sake of illustration that pre-shrunk yarn is used in the fabric, it may constitute all the warp yarns 18 and be as described in connection with the preceding figures or constitute all the filler threads 19 and be as described in connection with Fig. 4, or constitute a part of the warp or a part of the filler, or part of both.

In Fig. 8 a construction is shown where a yarn 12a, Fig. 3 may be used.

A fabric made entirely from pre-shrunk bast yarn is substantially shrink-proof, is stronger wet than dry, and withstands repeated washing and ironing with less wear and tear than known fabrics having the same denier and weight characteristics.

Fabrics made from any of the yarns herein described will have all or some portion of their surface composed of the fibrils 10 of the pre-shrunk fibre. The extent of said surface will depend upon the construction of the yarn which obviously depends upon the use of the fabric in which it is used, and the amount of it used in the fabric.

It would be difficult indeed to recite even a few of the combinations possible and it is not deemed necessary to do so in view of the fact that once the inventive concept herein disclosed is understood, it is merely a matter of selecting the amount of pre-shrunk fibrils 10 to be used in the staple or roving to make the yarns and the construction of the fabric using the selected yarn.

This specification employs the terms "shrink-proof," "comparatively shrink-proof" and "substantially shrink-proof" to describe that quality which is commonly termed "shrink-proof" found in rovings, yarns and fabrics that will shrink less than 2%. No fiber made today is absolutely "shrink-proof." However, American Standards

Association System has defined "shrink-proof" and "substantially shrink-proof" fabrics to mean that the shrinkage of such rovings, yarns or fabrics will be not more than 2%. This specification therefore employs these terms as they are commonly understood in this art.

As previously stated herein, the composition of the yarns (Figures 5 and 6) may be varied within wide limits, and by way of illustration, a cloth made of 30% of yarn (Figure 1 and Figure 5) of degummed and pre-shrunk linen fibers, and 70% viscose rayon (Figure 5) will not shrink or elongate more than .0136%, which is less than the 2% specified in the American Standards Association System referred to above. The same shrink-proof qualities apply to a 25% mixture of yarn (Figure 1) with 75% viscose rayon. As heretofore pointed out, the extent of this use of such pre-shrunk yarn (Figure 1) with other yarns can be varied within wide limits, and the shrink-proof quality of fabrics made therefrom may be varied accordingly.

Linen produced by the above described method has superior "ironability," a term used in the trade to denote that the goods will withstand high ironing temperatures, the pre-shrunk degummed fibers which are tubular and have cellular walls acting to insulate the other fibers interspun therewith and insulate them from heat. Cloth made from a mixture of 30% degummed and pre-shrunk linen fibers and 70% viscose rayon will shrink less than 2% when washed repeatedly or even boiled, and will withstand ironing temperatures of 300° to 350° F. without becoming tackey and without the iron sticking to the goods and without damage.

A common test for "ironability" is to place a cigarette paper on the goods and an approximately 350° F. iron thereto. With ordinary goods not containing the degummed and pre-shrunk fibers disclosed herein the paper is browned; the iron sticks to the goods. When the above rayon degummed linen mixture is used, the paper will brown but the iron will not stick to the goods because of the insulating qualities of the degummed pre-shrunk fibers.

As previously stated herein, a suitable method

of degumming and shrinking the bast fiber is referred to in the co-pending application Serial Number 103,262 which discloses a chemical degumming process, the bast fiber being immersed in a chemical bath until the desired amount of gum is extracted therefrom to permit the fibers to be dry-spun over standard cotton or woolen machinery as aforesaid. Obviously any method of degumming that will not remove the desired amount of gum to permit the fibers to be dry-spun cannot be employed. As stated in said co-pending application Serial Number 103,262, the exact degumming fluid employed and the time the fiber is immersed therein depends upon the character of the fiber.

What is claimed is:

A fabric having substantially non-shrinkable qualities, said fabric being composed of dry-spun yarns, said yarns being blended in part of staples of degummed and substantially completely pre-shrunk flax or hemp fibrils, and in part of other shrinkable fibrils.

ANTON F. BURKARDT.

25 References Cited in the file of this patent  
UNITED STATES PATENTS

| Number       | Name                       | Date          |
|--------------|----------------------------|---------------|
| 8,134        | Claussen -----             | June 3, 1851  |
| 9,650        | Pownall -----              | Apr. 5, 1852  |
| 30 679,695   | Ellis -----                | July 30, 1901 |
| 882,866      | Butterworth -----          | Mar. 24, 1908 |
| 1,313,594    | Hartshorne -----           | Aug. 19, 1919 |
| 1,607,220    | Von Ehrenthal et al. ----- | Nov. 16, 1926 |
| 1,986,970    | Haughey -----              | Jan. 8, 1935  |
| 35 2,070,273 | Haughey -----              | Feb. 9, 1937  |
| 2,122,175    | Coulter -----              | June 28, 1938 |
| 2,128,929    | Estes -----                | Sept. 6, 1938 |
| 2,230,269    | Pierce -----               | Feb. 4, 1941  |
| 40 2,260,229 | Nutter et al. -----        | Oct. 21, 1941 |
| 2,371,573    | Sabner -----               | Mar. 13, 1945 |
| 2,468,771    | Montonna et al. -----      | May 3, 1949   |

FOREIGN PATENTS

| Number     | Country             | Date          |
|------------|---------------------|---------------|
| 45 309,367 | Great Britain ----- | Apr. 11, 1929 |